

Patented Jan. 26, 1937

2,068,817

# UNITED STATES PATENT OFFICE

2,068,817

## COPPER ALLOY AMENABLE TO HEAT TREATMENT

Ulrich Raydt, Klaus Hanser, and Max Venzlaff,  
Osnabrück, Germany, assignors to Firma Osnabrücker Kupfer- und Drahtwerk, Osnabrück  
Germany, a firm of Germany

No Drawing. Application October 18, 1934, Serial  
No. 748,965. In Germany October 18, 1933

2 Claims. (Cl. 148—21.2)

It is known to make additions of manganese, cobalt and chromium either separately or several at a time to pure copper or to copper alloys, for example tin bronzes. Alloys of most varied composition containing these constituents are used for many different purposes. The said additional substances improve the properties of the alloys in various respects. The alloys, however, with the exception of copper-chromium alloys are not amenable to heat treatment.

By means of the present invention it is possible to make these alloys amenable also to heat treatment and to obtain values for the tensile strength and hardness which far exceed the values for the corresponding hitherto known alloys which were not responsive to heat treatment. The alloys are made responsive to heat treatment by an addition of phosphorus in the proportion of about 0.1% or more in addition to the above mentioned additions of manganese, cobalt and chromium. The upper limit of the phosphorus content is determined by the capability for being worked which the alloys are to possess.

Manganese, cobalt and chromium may be present in the alloy either separately or two or more of them may be present at the same time. The total content of these metals should not be less than 0.2%, if the alloy is to be amenable to heat treatment. There is no upper limit to the content of these additional metals in the alloy, and they may be present in far greater proportions than corresponds to the phosphorus content having regard to the fact that the property of being amenable to heat treatment is probably due to the effect of the corresponding metallic phosphide, such as for example  $Mn_5P_2$ . The alloys can also contain tin, zinc and other of the usual constituents of copper alloys. Iron also has an advantageous effect as is otherwise usual.

The new alloys can be heat-treated by heating them to a temperature above 700° C., quenching and ageing at 400–600° C. The heat treatment can also be carried out by heating the alloys to temperatures above 700° and then gradually cooling them. In this way values are obtained for the tensile strength and hardness of the alloys which exceed the values obtained for the quenched alloys but are, in general, less than the values obtained when the heat treatment consists of heating, quenching and ageing. The alloys which have been cooled down slowly can, however, also be tempered in the same manner as the quenched alloys, in which case approximately the same values are obtained as for the quenched and in the tempered pieces.

Cast alloys as well as alloys capable of being formed plastically, for instance, by rolling or drawing, are amenable to the heat treatment. The latter can be subjected after the forming and before the tempering or even after the heat treatment has been completed, to a subsequent cold treatment whereby known increases in tensile strength, hardness etc. are obtained though the elongation is simultaneously reduced.

The improved qualities possessed by the new alloys will be seen from the following comparative figures for the tensile strength, hardness and elongation.

An alloy containing 2% of manganese in the cooled condition had a tensile strength of about 25 kg./mm.<sup>2</sup> with an elongation of 45% and a Brinell hardness of 61 kg./mm.<sup>2</sup>. When this alloy was subjected to heat treatment as above described these figures did not alter in any way. When 0.15% of phosphorus was added to the same alloy, a test sample quenched from 800–900° C. had a tensile strength of 26 kg./mm.<sup>2</sup>, an elongation of somewhat over 40% and a Brinell hardness of 65–70 kg./mm.<sup>2</sup>. When this alloy was tempered at about 500° C., the tensile strength rose to about 36 kg./mm.<sup>2</sup> and the Brinell hardness to 110–120 kg./mm.<sup>2</sup>, while the elongation fell to about 20%. When the quenching process was omitted in the case of this alloy and the alloy was allowed to cool down naturally from 800–900° C., the value for the tensile strength was about 30 kg./mm.<sup>2</sup>. When this naturally cooled sample was tempered almost the same figures were obtained as those indicated previously for the quenched and tempered sample.

In the case of an alloy containing 0.6% manganese and 0.3% phosphorus as well as 1.8% tin and 0.15% iron and subjected to heat treatment a tensile strength of about 45 kg./mm.<sup>2</sup> and a Brinell hardness of 130–140 kg./mm.<sup>2</sup> were obtained with an extension of about 30%.

What we claim is:—

1. An age hardened copper base alloy, free of beryllium, containing not less than 0.2% of manganese and from 0.1 to 0.5% phosphorus characterized by the fact that the age hardening is due primarily to the combined effect of the manganese and phosphorus.

2. An age hardened copper base alloy free of beryllium, containing about 0.6% manganese, about 0.3% phosphorus, from 1 to 2% tin, and 0.1% to 0.2% iron, the remainder being copper.

ULRICH RAYDT.  
KLAUS HANSER.  
MAX VENZLAFF.

55